

# UNITED STATES PATENT OFFICE.

EDWARD DROULARD, OF RIVER ROUGE, MICHIGAN.

## LEATHER-DRESSING.

1,278,886.

Specification of Letters Patent. Patented Sept. 17, 1918.

No Drawing.

Application filed October 29, 1917. Serial No. 199,180.

To all whom it may concern:

Be it known that I, EDWARD DROULARD, a citizen of the United States of America, residing at River Rouge, in the county of Wayne and State of Michigan, have invented 5 certain new and useful improvements in Leather-Dressings, of which the following is a specification.

This invention relates to a liquid dressing 10 or lubricator for leather, and the object of my invention is to provide a liquid composition that may be applied to leather or similar material to polish, preserve and soften the leather and to increase the longevity of 15 the same.

I attain the above object by a liquid composition that has been especially compounded for leather belts and the composition includes ingredients which will polish the belt, 20 exclude foreign matter from pores or interstices of the belt, and increase the pliability and consequently its adherence to a wheel about which the belt is trained.

The composition includes turpentine, rosin, 25 castor oil, coal oil and pitch, and for compounding three gallons of the liquid dressing, it is preferable to use the following portions or approximately so:

|                      |                   |
|----------------------|-------------------|
| Roofing pitch or tar | 1 gallon.         |
| Coal oil or kerosene | 1 gallon plus.    |
| Turpentine           | ½ cup.            |
| Rosin                | 2 pounds.         |
| Castor oil           | 6 tablespoonfuls. |

Enough coal oil or kerosene is added to 35 the roofing pitch or tar to dissolve the same so that the pitch or tar will be in liquid form. This ingredient is employed to fill the pores or interstices of a leather belt and to 40 exclude dirt and water.

The turpentine is included to add a polish to a belt and increase the pliability of the same, while the rosin will cause the belt to adhere and snugly engage the wheel about which the belt is trained, thereby increasing 45 the efficiency of the belt as a power transmitting element.

The castor oil is used for the same purpose as the rosin particularly in a high grade of leather dressing, but in a low 50 grade of dressing, it may be left out.

After the coal oil or kerosene has dissolved the pitch or tar, the other ingredients are added and the entire admixture boiled for about five minutes, allowed to 55 cool, and is then ready to be used as a leather dressing.

What I claim is:—

1. A liquid dressing for leather comprising tar, kerosene, turpentine, rosin and castor oil. 60

2. A liquid dressing for leather comprising tar, kerosene, turpentine and rosin.

3. A liquid dressing for leather comprising one gallon of tar, one and a half gallons 65 of kerosene, half a cup of turpentine, two pounds of rosin, and six tablespoonfuls of castor oil.

4. A liquid dressing for leather comprising one gallon of tar, one and a half gallons 70 of kerosene, half a cup of turpentine, and two pounds of rosin.

In testimony whereof I affix my signature in the presence of two witnesses.

EDWARD X DROULARD.  
his  
mark

Witnesses:

LEWIS E. FLANDERS,  
ANNA M. DORR.